

July 2, 1935.

J. J. BLUM

2,006,626

FELTED FIBROUS PRODUCT AND METHOD OF MAKING SAME

Filed April 24, 1933

Fig. 1.



Fig. 3.



Fig. 2.



Fig. 5.



Fig. 4.



Inventor:  
Jerome J. Blum,  
By Frank L. Belknap,  
Attorney.

## UNITED STATES PATENT OFFICE

2,006,626

FELTED FIBROUS PRODUCT AND METHOD  
OF MAKING SAMEJerome J. Blum, Olean, N. Y., assignor to Arvey-  
ware Corporation, Olean, N. Y., a corporation  
of Delaware

Application April 24, 1933, Serial No. 667,687

2 Claims. (Cl. 92—55)

This invention relates to improvements in a felted fibrous product and a method of making the same, and refers specifically to a felted fibrous product having integrally united to a surface thereof a textile fabric, and a method of forming and uniting the fibrous material to the fabric.

It is frequently desirable, in the use of felted fibrous products to have a textile fabric secured to the surface of the fibrous article. This object has heretofore been accomplished by adhesively uniting cloth or other textile fabric to the fibrous base. However, serious difficulties and disadvantages attend the manufacture and use of such a product. For example, in the use of the product the adhesive used may be detrimentally influenced by heat, cold or moisture to release the bond between the fibrous base and the fabric which, of course, is most undesirable, limiting the selection of adhesives which are suitable for use and also limiting the purposes and conditions under which the product may be used. In manufacturing, serious difficulties are presented, particularly where the product takes irregular shapes or forms such as the felted fibrous liners for dashboard or instrument board compartments upon automobiles. Due to the peculiar and varying shapes required by the automotive industry so as to obtain the largest possible compartment space while avoiding interference with other parts which are necessarily attached to and under the dash, the curves and angles presented in the compartment are of such a nature as to render it almost impossible to obtain a good fitting textile lining when the lining is to be adhesively attached. This task, of course, must be performed manually and is tedious, time consuming and expensive.

To obviate the difficulties hereinbefore set forth and to produce a felted fibrous article or product having an integrally attached cloth or fabric lining which will not become detached from the fibrous base by heat, cold or moisture, is an object of my invention.

Briefly described, the process of my invention comprises, positioning upon the usual foraminated felting form a sheet or web of cloth or fabric, cut sewed and fit to the shape of the form, if said form is such as to make a fibrous container or compartment liner of more or less irregular shape. The form carrying the fabric lining may then be immersed in a bath of fibrous pulp and a condition of vacuum may be established within the form in the conventional manner. Fibrous material from the pulp is thus deposited upon the form and the fibres interlock and intertwine

with the lint, or nap of the fabric, thereby integrally securing the fabric to the deposited fibres. When a desired thickness of fibres has been deposited, the form may be removed from the pulp bath and the deposited fibres subjected to a repressing action by means of the usual "rubber hat" method. The vacuum may then be released and air under pressure may be introduced into the form to remove the fibrous product.

The fabric lining, of course, being cut and sewed to fit the form, in the finished product conforms precisely with the contour of the fibrous product regardless of the irregular curves, angles or crevices comprised in the product. Further, it is substantially impossible to remove fabric from the fibrous base without destroying the base, since it is substantially an integral portion of the base itself. In addition, the integrally united fabric serves to strengthen the base against such stresses as tension, bending or the like.

Other objects and advantages of my invention will be apparent from the accompanying drawing and following detail description.

In the drawing, Fig. 1 is a fragmentary top plan view, parts being broken away of a felting form carrying a portion of the product comprising my invention.

Fig. 2 is a sectional view taken on the line 2—2 of Fig. 1.

Fig. 3 is an enlarged fragmentary sectional view similar to Fig. 2, illustrating particularly the interlocking engagements of the fibres and fabric.

Fig. 4 is a perspective view of a felted fibrous liner utilized as a dashboard compartment, the liner having an integrally united fabric lining.

Fig. 5 is a transverse sectional view taken on line 5—5 of Fig. 4.

Referring in detail to the drawing, 1 indicates the body portion of a conventional felting form which is usually constructed of metal and is provided with a plurality of slots or grooves 2 opening to one face thereof. A plurality of apertures 3 may connect grooves 2 to the opposite face of the member 1, said apertures being provided to drain off the aqueous carrier of a fibrous pulp under the influence of vacuum. The member 1, although being illustrated in the drawing as a flat planar surface, may take any desired shape or form depending upon the shape or form of the fibrous article or product to be felted.

A plate 4, usually constructed of metal, and provided with a plurality of perforations 5 may

be positioned upon the member 1 adjacent that face of said member provided with the grooves or slots 2. A major portion of the perforations 5 communicate with the grooves 2 whereby the aqueous carrier of the pulp solution may pass through perforations 5 under the influence of vacuum. By the provision of plate 4 a relatively smooth uniform surface is obtained. A relatively fine gauge wire screen 6 may be positioned upon plate 4 whereby the condition of vacuum established at the rear face of the member 1 may be uniformly effectively established over the entire surface.

In the manufacture of the usual felted fibrous products the apparatus thus far described may be immersed in a fibrous pulp and a condition of vacuum established at the rear face of the member 1. It can readily be seen that, the aqueous carrier of the fibrous pulp may be freely drawn through screen 6, plate 4 and apertures 3. However, the fibres constituting the pulp solution are prevented from passing through screen 6 and consequently the same are deposited upon said screen to a desired depth dependent upon the character of the product being manufactured. When a desired thickness of fibres has been deposited upon screen 6, the form comprising member 1, plate 4, screen 6 carrying the deposited fibres, is removed from the pulp bath and, depending upon the surface characteristics of the product desired, the deposited layer of fibres may be subjected to a pressing action or other treatment. Subsequently, air under pressure may act from the rear face of member 4 to dislodge the fibrous layer from screen 6.

As a feature of my invention, I contemplate the disposition of a sheet or web of fabric 7 upon screen 6 prior to the immersing of the form in the pulp bath. It can readily be seen that when the form carrying the fabric sheet or web 7 is immersed in the pulp and a condition of vacuum established at the rear face of member 1, the aqueous carrier of the pulp will be drawn through the interpositioned web 7 and the individual fibres constituting the pulp will be deposited upon the fabric web instead of screen 6. When a desired thickness of fibres has been deposited upon the fabric 7, the form may be removed from the pulp bath with a layer 8 of fibres carried upon the fabric web 7. If desired, while the felted layer 8 is still carried upon the form, said fibrous material may be subjected to a pressing action by the process commonly known to the art as the "rubber hat" method. In this manner the surface of the fibrous body may be smoothed or otherwise finished as desired. The vacuum may then be released and a condition of pressure may be established to blow off or otherwise remove the fibrous structure carrying the fabric web from the form.

It can readily be seen that, a different condition exists between depositing the fibres upon a metallic screen such as screen 6 and depositing said fibres upon the fabric web 7. Screen 6 comprises a plurality of woven reticulated wires the surfaces of which are relatively smooth whereas the individual strands constituting the fabric has a more or less "fuzzy" surface, the various strands when woven to form the fabric, producing a web 70 having a more or less "linty" surface. When

the fibres are deposited upon the screen 6 no bond is established between the individual wires constituting the screen and the fibres constituting the fibrous layer. However, when the fibres are deposited upon the "linty" surface of fabric 7 the individual fibres constituting the fibrous layer intertwine or interlock with the lint of nap upon the surface of the fabric to integrally unite the fabric 7 to the fibrous layer 8, as shown best at 9 in Fig. 3.

Referring particularly to Figs. 4 and 5, a felted fibrous liner 10 is shown which may be utilized to define a dashboard or instrument board compartment upon an automobile, the open portion 11 of the liner being positioned adjacent the surface 15 of the dashboard which latter is usually provided with a door. It is desirable, of course, to line the inside of such a compartment with a textile fabric in order to impart a finished appearance thereto and also to prevent scratching or marring of articles of a delicate nature which may be positioned within the compartment. It is well known that, most available space upon an automobile is utilized to advantage, particularly adjacent and under the dashboard of the machine. Hence, it becomes necessary to construct the compartments in peculiar shapes or forms in order to avoid interference with instruments, wires, and like necessary equipment. For instance, the section contour of the liner 10 may be of the irregular sectional shape shown at 12 in Fig. 5 which section may not be uniform throughout the length of the liner. A liner of this character may be constructed very easily and economically by utilizing the concepts of my invention inasmuch as the only additional steps necessary in the process of making the ordinary unlined liner are that a fabric bag be cut, sewn and fitted to the form upon which the usual liner is to be felted. The felting operation is then carried out in the manner hereinbefore described and the lining of the resulting product, being formed as an integral portion of the liner itself, fits perfectly within the liner and is substantially non-destructible in regard to its tearing from the surface of the liner. It can readily be seen that in order to manually adhesively unite a cloth lining similar to lining 13 within the liner 10 and to perform a neat, finished and efficient job would be a tedious, a time consuming and expensive task.

I claim as my invention:

1. A preformed, felted, relatively rigid fibrous structure having curvilinear surfaces, one external surface of said structure comprising a linty fabric sheet, the lint of which is intertwined with the fibres comprising said structure.

2. In a process wherein the aqueous carrier of a fibrous pulp is passed through a receptacle-shaped foraminated surface under the influence of vacuum, to deposit a relatively thick layer of fibres upon said surface, to produce a relatively rigid fibrous structure, the improvement which comprises, disposing a linty fabric web conforming in contour with said surface upon said surface prior to the passage of the carrier therethrough whereby to intertwine the fibres and the lint of the fabric to unite said fabric to the fibrous structure and thereby form an integral unit.